

March 11, 1947.

T. H. SLOAN

2,417,328

METHOD OF MAKING GLASSWARE

Filed Jan. 27, 1944

3 Sheets-Sheet 1

*Fig.1.*



*Fig. 1B.*



*Fig. 1A.*



*Fig. 2.*



INVENTOR

Theodore H. Sloan

by his attorneys  
Stebbins, Blenko & Webb

March 11, 1947.

T. H. SLOAN

2,417,328

METHOD OF MAKING GLASSWARE

Filed Jan. 27, 1944

3 Sheets-Sheet 2

*Fig. 2A.*



*Fig. 3.*



*Fig. 4.*



*Fig. 2B.*



INVENTOR

Theodore H. Sloan

by his attorneys

Stebbins, Blenks & Webb

March 11, 1947.

T. H. SLCAN

2,417,328

METHOD OF MAKING GLASSWARE

Filed Jan. 27, 1944

3 Sheets-Sheet 3

*Fig. 5.*



*Fig. 6.*



*Fig. 7.*

INVENTOR

Theodore H. Sloan

BY

Stebbins, Blenko & Webb

HIS ATTORNEYS

## UNITED STATES PATENT OFFICE

2,417,328

## METHOD OF MAKING GLASSWARE

Theodore H. Sloan, Charleroi, Pa., assignor to  
 G. M. S. Corporation, Pittsburgh, Pa., a corporation of Pennsylvania

Application January 27, 1944, Serial No. 519,878

9 Claims. (Cl. 49—85)

1

This invention relates to the manufacture of glassware and particularly to the making of footed ware such as goblets, stem-foot ware, and the like.

So far as I am aware, no satisfactory method of producing footed goblets or like stemware by pressing in one piece has been known heretofore, except those involving hand operations. Such footed ware as has been pressed in one piece by hand heretofore has been characterized by objectionable seams extending up to the rim and down to and around the edge of the foot. I have invented a novel method of making footed ware such as stem-foot goblets having a bowl which is without seams, by a series of operations which may readily be performed by a rotary-table press machine.

In a preferred practice of the invention, I employ a mold including an upper portion providing a cavity for forming the rim or lip and upper part of the bowl of the ware, and a lower portion providing cavities for forming the bottom of the bowl and the foot, and a constriction between the cavities for forming the stem or foot connection. Both portions of the mold may be segmental but the upper portion is preferably a continuous ring. The lower portion of the mold is open at the bottom and is engraved to provide a design on the exterior of the ware which effectively conceals seams formed at the joints between the segments of the mold. After placing a mass or gob of molten glass in the mold, I apply fluid pressure above the glass to force a portion thereof through the stem portion of the mold to fill the latter and form a spherical mass of glass as an appendage on the main mass at the open bottom of the mold. I limit the amount of glass flowing through the stem portion of the mold cavity by preforming the appendage to a definite size under suction, if needed.

On completion of these several steps, a forming plunger is applied to the spherical appendage of glass at the bottom of the stem, and pressure exerted thereon, thus shaping the foot or base of the ware. I then shape the balance of the glass remaining in the top portion of the mold into the bowl of the ware by means of a press plunger. This operation completes the formation of one goblet or piece of other stem-foot ware. The mold or the segmental lower portion thereof at least, is then expanded and the finished ware is lifted out of the mold.

Other novel features and advantages of the invention will become apparent during the following detailed description and explanation which

2

refer to the accompanying drawings illustrating the several steps of the method of my invention.

In the drawings,

Figure 1 is a section through a mold showing the charge or gob of molten glass as initially deposited therein;

Figure 1A is a similar view showing the blowing of a portion of the gob through the mold to form the finished stem, and the preliminary shaping of the portion of the glass which eventually is to form the foot;

Figure 1B is a view similar to Figure 1 showing the glass in condition for the pressing of the foot;

Figure 2 is a view similar to Figure 1 showing the actual shaping of the foot;

Figure 2A is a view similar to Figure 1 showing the shaping of the bowl portion and foot;

Figure 2B is a view similar to Figure 1 showing the goblet in the mold after final shaping;

Figures 3 and 4 are additional views similar to Figure 1 showing succeeding steps in the operation which will be fully described and explained hereinafter; and

Figures 5 through 7 are perspective views of other forms of ware which may be produced by my method.

Referring now in detail to the drawings, a plurality of molds are mounted on a press-machine table 11. The table 11 is adapted to be rotated in a step-by-step manner so that the molds advance successively from one station to the next, around the periphery of the table, for the performance of the several operations about to be described. The description will cover the progress of one mold through each of the several stations occupied by the molds but it will be understood that the same operation is performed at any given station upon all the several molds, in the manner of operation characteristic of rotary machines for making glassware.

One of the molds 10 is illustrated in detail in Figures 1 through 4, which show the several steps of the complete manufacturing operation. Each mold includes a base plate 12 mounted on the machine table 11. A mold housing 13 resting on the plate 12 supports a mold portion 14 adapted to shape the upper portion of the bowl of the ware. In the mold illustrated, the portion 14 is a continuous or one-piece top ring. It may, however, be segmental. The lower portion 15 of the mold is composed of a plurality of segments movable radially within the housing 13. The segments have a slot and shoulder connection 16 with the lower portion of the ring 14. The

bottoms of the segments of the mold portion 15 rest on a base ring 17 carried on the plate 12. The base 12 and the base ring 17 have central openings therein in alignment with a hole 18 through the table 11. The segments when contracted define cavities for forming the lower portion of the bowl of a piece of ware and the foot, with a constriction therebetween for forming the stem or foot connection.

As shown in Figure 1, the segments of mold portion 15 are contracted at the first station. When the mold is at this station, a gob of molten glass 19 is dropped through the ring 14 and into the lower mold portion 15. If the ring 14 is segmental, its segments are, of course, contracted before the gob is dropped. While the mold dwells at the first station a blowhead 20 is lowered at thereon and a preforming plunger 21 is raised into contact with the lower portion of the mold, as shown in Figure 1A. Air under pressure is admitted through a pipe 22 and a passage 23 in the head to the interior of the mold above the gob. Simultaneously suction may, if needed, be applied to the lower portion of the mold by a passage 24 through the plunger 21. The upper end of the plunger 21 is shaped to form a spherical appendage 25 on the main mass of glass as a portion thereof flows through the open bottom of the mold. The amount of glass flowing through the mold, however, is definitely limited by the plunger 21. The appendage 25, of course, is connected to the remainder of the glass by a stem or foot connection 25a formed in the bottom of the mold portion 15.

The gob begins to set up immediately on contact with the mold, as a result of the loss of heat thereto. After a time sufficient to permit the glass flowing through the mold to fill the recess in the top of plunger 21, the blowhead 20 is raised and the plunger 21 is lowered leaving the glass in the mold in the condition illustrated in Figure 1B. It is to be noted that the appendage 25 is substantially spherical in shape. It thus tends to retain sufficient heat so that it may easily be molded to form the foot, in the manner now to be described. After the preforming of the foot, as illustrated in Figures 1A and 1B, the table 11 is advanced one step, bringing the mold to the second station. When at that location, a plunger 26 is raised to press the appendage 25. As shown in Figure 2, the upper end of the plunger 26 is shaped to form a foot 27 on the partly formed piece of ware. As a result of the air pressure applied by the blowhead 20, the glass fills the lower portion of the mold, insuring that the stem or connection 25a between the foot and the bowl of the ware is fully filled out. The preforming of the appendage 25 insures that just the right amount of glass is available to form the foot. The edge of the finished foot is thus kept free from the mold segments so that no seams are formed thereon.

While the mold remains at the second station, a bowl-forming plunger 28 is brought down through the ring 14 to press the remainder of the glass upwardly into a complete bowl 31 as shown in Figure 2A. A collar 29 on the plunger 28 has a groove 30 effective to shape the rim of the goblet bowl. When the goblet has been completely shaped, the plungers 26 and 28 are withdrawn leaving the piece of ware in the mold in the condition shown in Figure 2B. The table next moves forward again to carry the mold to the third station.

At the third station a nozzle 32 delivers a cooling

blast of air into the ware from above, as shown in Figure 3. After the preliminary cooling at the third station, the mold is advanced by another step to the fourth station. At that point, as shown in Figure 4, the segments of the lower mold portion 15 are "cracked" or slightly expanded and streams of cooling air are delivered onto the ware from above and below by nozzles 33 and 34, respectively. "Cracking" of the lower mold portion permits longitudinal contraction of the ware. It will be observed that the ware remains suspended in the ring 14 which, being continuous, is not capable of enlargement. If the ring 14 were segmental, it would preferably be held contracted at this stage. The opening of the lower mold portion also aids cooling of the ware. On the next movement of the table, the mold is advanced to the fifth station at which the foot and stem of the ware are further cooled by a stream of air from a nozzle.

After final cooling at the fifth station the mold advances with the next movement of the table to the sixth station at which the lower mold portion is fully opened. A lifting plunger is moved upwardly through the table and mold and is effective to raise the ware into elevated position for engagement by a take-away mechanism. By means of a passage through the plunger, suction may be applied to the foot of the piece of ware to aid in holding it on the plunger. It will be noted that the minimum inside diameter of the ring 14 is sufficiently greater than the maximum diameter of all portions of the ware formed by the lower mold portion to permit this upward removal of the ware through the ring. When the ware has been engaged by the take-away mechanism, the plunger is lowered and the table is again moved forward to advance the mold to subsequent stations for further cooling, closing and oiling.

Figures 5, 6 and 7 show other typical forms of ware which may be made by my method, in addition to that shown in Figure 4.

It will be apparent from the foregoing description that the invention provides a highly advantageous method of shaping footed glassware by pressing a charge of molten glass in a mold. The exact amount of glass needed to form the foot is positively forced through the mold by air pressure and preformed to a heat-retaining shape. If a continuous ring is used for the upper portion of the mold the upper portion of the ware may be formed without seams. The portion of the bowl formed by the segmental portion or portions of the mold may be fluted or otherwise embellished, as shown in the drawings, thereby effectively concealing the seams formed at the joints between the segments composing the mold. The formation of the bottom of the foot by a plunger and the preforming of the foot eliminates seams on the lower side and edge of the foot.

The invention thus provides a satisfactory method whereby footed ware having a seamless bowl may be formed by a press machine. It will also be noted that the ware is fully finished in a single mold. The invention is particularly well suited to the production of light-walled ware.

While I have disclosed herein but a preferred practice of the invention, it will be understood that changes in the specific operations described may be made without departing from the spirit of the invention or the scope of the appended claims.

I claim:

1. In a method of making footed glassware in

a mold having a bowl-forming cavity in a portion thereof at least a part of which is in one piece, and stem-forming and foot-forming cavities in mold portions which are segmental, the steps including dropping a mass of molten glass into the mold, applying fluid pressure above the mass and simultaneously confining the glass flowing through the stem-forming cavity into the foot-forming cavity to preform it into a generally spherical appendage, pressing the appendage to form a foot and pressing the glass in the bowl-forming cavity to form the bowl.

2. In a method of making footed glassware, the steps including dropping a mass of molten glass through a one-piece mold portion having therein a part, at least of a cavity for forming the bowl of the ware, into segmental mold portions having therein cavities for forming the remainder of the bowl, the stem and the foot, applying fluid pressure above the mass and simultaneously confining the glass flowing through the stem-forming cavity into the foot-forming cavity to preform it into a generally spherical appendage, pressing the appendage to form a foot and pressing the glass in the bowl-forming cavity to form the bowl.

3. In a method of making footed glassware, the steps including dropping a mass of molten glass into a mold having cavities for forming a bowl, stem and foot, applying fluid pressure above the mass and suction therebelow to force a portion thereof through the stem-forming cavity and into the foot-forming cavity, pressing the glass in the foot-forming cavity into a foot, and pressing the remainder of the glass into a stem and bowl.

4. In a method of making footed glassware, the steps including dropping a mass of molten glass into a mold having cavities for forming a bowl, stem and foot, applying fluid pressure to the mass to force a portion thereof through the stem-forming cavity and into the foot-forming cavity, preforming the glass in the foot-forming cavity into a generally spherical appendage, pressing the appendage into a foot, and pressing the remainder of the glass into a stem and bowl.

5. In a method of making footed glassware, the steps including dropping a mass of molten glass into a mold having cavities for forming a bowl, stem and foot, applying fluid pressure to the mass to force a portion thereof through the stem-forming cavity and into the foot-forming cavity, preforming the amount of glass flowing into the foot-forming cavity and then pressing it into a foot while pressing the remainder of the glass into a stem and bowl.

6. In a method of making footed glassware, the steps including dropping a mass of molten glass into a mold having cavities for forming a bowl, stem and foot, applying fluid pressure to the mass to force part of it through the stem-

forming cavity and pressing said part into a foot while pressing the remainder of the glass into a stem and bowl.

7. In a method of making a glass article including a bowl, stem and foot in a mold having segments providing cavities for forming the stem and foot, and a one-piece portion providing a cavity for forming the bowl, the steps including dropping a mass of molten glass into the bowl-forming cavity of the mold, introducing a foot-preforming member into the foot-forming cavity while forcing a portion of the glass by pneumatic pressure through the stem-forming cavity to preform an appendage of glass of predetermined size, and then simultaneously pressing the appendage and the glass in the bowl-forming cavity to give final shape thereto.

8. In a method of making footed glassware, the steps including dropping a mass of molten glass into a mold having cavities for forming a bowl, stem and foot, the mold portion forming the cavities for the stem and foot being segmental, applying fluid pressure to the mass to force part of it through the stem-forming cavity, preforming the amount of glass which flows into the foot-forming cavity and pressing it into a foot while pressing the glass in the bowl-forming cavity into a bowl, and controlling the pressing of the foot to limit the spreading thereof and prevent contact of the edge thereof with the mold.

9. In a method of making a footed goblet or the like having a seamless bowl, the steps including dropping a mass of glass through a one-piece mold portion having a bowl-forming cavity therein and into a segmental mold portion having stem-forming and foot-forming cavities therein, applying fluid pressure on the mass to force a portion thereof through the stem-forming cavity, confining said portion thereby forming it into an appendage, pressing the appendage to form a foot and pressing the remainder of the glass to form a stem in the segmental mold portion and a seamless bowl in said one-piece mold portion.

THEODORE H. SLOAN.

#### REFERENCES CITED

The following references are of record in the file of this patent:

#### UNITED STATES PATENTS

| Number    | Name     | Date          |
|-----------|----------|---------------|
| 2,070,493 | Rosa     | Feb. 9, 1937  |
| Re. 5,924 | Reighard | June 16, 1874 |
| 567,236   | Hilde    | Sept. 8, 1896 |
| 2,276,399 | Hrdina   | Mar. 17, 1942 |

#### FOREIGN PATENTS

| Number  | Country | Date          |
|---------|---------|---------------|
| 488,603 | British | July 11, 1938 |